

Oct. 23, 1951

2,572,783

BAREND GYSBERTUS HENDRIKUS VAN DER JAGT  
NOW BY CHANGE OF NAME  
BAREND GYSBERTUS HENRY VANDERJAGT  
PROCESS OF PRODUCING A SPINNABLE SLIVER  
Filed July 20, 1946



SCRUB PALMETTO STEM

CUT INTO LOGS → MECHANICAL DEFIBRATION → SEPARATION INTO → LONG FIBERS (MORE THAN 5 INCH)      SHORT FIBERS (LESS THAN 5 LONG)

Boiling for  $\alpha$  hours  
in caustic Soda Solution  
of  $b^{\circ}$  Be'  
( $\alpha \times b = 5$  to 12)

SLIVER FORMATION

→ WASHING → DRYING →

BROWNISH  
SPINNABLE  
FIBER

FIG. 5.

INVENTOR  
BAREND GYSBERTUS HENDRIKUS VAN DER JAGT,  
NOW BY CHANGE OF NAME,  
BAREND GYSBERTUS HENRY VANDERJAGT

BY   
HIS ATTORNEY

## UNITED STATES PATENT OFFICE

2,572,783

## PROCESS OF PRODUCING A SPINNABLE SLIVER

Barend Gysbertus Hendrikus Van der Jagt,  
Washington, D. C.; now by change of name,  
Barend Gysbertus Henry Vanderjagt

Application July 20, 1946, Serial No. 685,018

5 Claims. (Cl. 19—66)

1

This application is a continuation-in-part of my copending application Serial No. 507,924, which was filed on October 23, 1943, and became abandoned on September 20, 1946, as a continuation-in-part of my application Serial No. 450,989, filed on July 15, 1942, and abandoned on December 30, 1943.

The present invention relates to a brownish spinnable sliver and to a process of producing such sliver from fibers obtained by a mechanical defibration of the stems of scrub palmetto plants. These plants grow abundantly in Florida and are also found in other parts of the continental United States and in the West Indies. The botanical name of the scrub palmetto plant is "*Serenoa repens*." The part of the scrub palmetto plant from which the fibers to be treated according to the present invention are obtained grows in a substantially horizontal direction underground and, for this reason, it was previously believed to be part of the root of the plant and identified as such in my application Serial No. 507,924 above referred to. However, according to recent information supplied by the U. S. Department of Agriculture, this underground part of the scrub palmetto plant is botanically its stem, and, consequently, it is identified as a stem in the present application.

Palmetto stem fibers as obtained by mechanical defibration of scrub palmetto stems are coarse, smooth, straight and highly elastic hard fibers which heretofore have been used only to a very limited extent in the manufacture of bristle brushes. In the form in which these fibers are obtained from mechanical defibration processes they have a light straw-yellow color, but these fibers cannot be formed into a sliver by sliver-forming machines because the coarse straight fibers tend to repel one another due to their great stiffness and resiliency.

In order to permit the formation of spinnable slivers on sliver-forming machines, it is necessary that the fibers supplied to such machine have a certain amount of cohesion which permits the fibers to be re-arranged lengthwise of one another by the machine and which causes the fibers to cohere in any re-arranged position. This property is completely lacking in fibers obtained from a mechanical defibration of the stems of scrub palmetto plants.

One object of the present invention is to produce from fibers obtained by a mechanical defibration of stems of scrub palmetto plants (*Serenoa repens*) a spinnable sliver.

In an application Ser. No. 685,017, now aban-

doned, filed concurrently herewith, a process is described and claimed for producing a light straw-colored spinnable sliver from fibers obtained by a mechanical defibration of the stems of scrub palmetto plants, said process including the steps of separating the mixture of long and short fibers obtained from a mechanical defibration of scrub palmetto stems into short fibers up to 5 inches length and longer fibers, tackifying the longer fibers, and forming the fibers into a sliver while they are in tacky condition. This sliver-forming process according to my concurrently filed application is not applicable to the short fibers of less than about 5 inches length.

It is, therefore, a specific object of the present invention to produce a spinnable sliver from scrub palmetto stem fibers of less than about 5 inches length.

The present invention is based on the discovery that short or long palmetto stem fibers when boiled with caustic soda solution of a certain limited strength for a certain limited time and then washed and dried will develop, on drying, hook-shaped kinks of a type not ordinarily formed in textile fibers as a result of treatments with caustic lyes, said hook-shaped kinks causing adjacent fibers to cohere together while being slidably displaceable lengthwise of one another and thus rendering possible the subsequent formation of a spinnable sliver on a sliver-forming machine.

Accordingly, the above mentioned objects of my invention are accomplished by a process which comprises the steps of boiling fibers obtained by a mechanical defibration of the stems of scrub palmetto plants (*Serenoa repens*) for a period ranging from about 10 minutes to about 2 hours in an aqueous caustic soda solution of between about 4° and about 55° Bé. strength, the strength of the solution being related to the boiling time according to the formula  $a \times b = 5$  to 12, where  $a$  is the boiling time in hours and  $b$  is the strength of the solution in degrees Bé., washing the fibers with an aqueous medium having a pH value between about 5.5 and 7, drying them, the fibers developing, during the drying, hook-shaped kinks causing adjacent fibers to cohere together while being slidably displaceable lengthwise of one another, and finally forming the kinky fibers on a sliver-forming machine into a spinnable sliver.

The aqueous medium used for washing the fibers after completion of the caustic lye boiling step may be cold or warm water. The water may be adjusted to a pH value between about 5½ and 7 by addition of a suitable acid, such as hydro-

## 3

chloric acid or acetic acid, to effect neutralization of any alkali remaining in the fibers.

The following examples describe several embodiments of the invention, reference being had to the accompanying drawings, in which:

Fig. 1 illustrates, somewhat diagrammatically, a group of fibers as obtained by a mechanical defibration of the stems of scrub palmetto plants;

Fig. 2 illustrates diagrammatically the same group of fibers after treatment in accordance with my invention prior to the formation of the sliver;

Fig. 3 illustrates diagrammatically a sliver formed from the treated fibers according to Fig. 2;

Fig. 4 shows a sliver formed according to the invention from scrub palmetto stem-fibers having a length up to 5 inches; and

Fig. 5 is a flow diagram of the process of producing a sliver of the type shown in Fig. 4.

## Example I

The stems of scrub palmetto plants (*Serenoa repens*), as dug up from the ground, were cut into equal lengths of about 14 inches, and the resulting logs were mechanically defibrated in a twilly devil. The resulting fibers were coarse, smooth, and substantially straight as illustrated at 10 in Fig. 1. They had a light straw color.

50 kg. of these fibers were placed in a vat containing a caustic soda solution of 15° Bé. strength and boiled in the solution at atmospheric pressure for 30 minutes. At the end of this period the fibers, the original light straw color of which had darkened to a brownish shade, were removed from the vat, washed with cold water, and left to dry. During the drying the fibers developed a peculiar type of hook-shaped kinks as indicated in Fig. 2.

These kinky fibers were fed to a sliver-forming machine and it was found that adjacent fibers would hook loosely on to each other by their kinks, permitting mutual displacement lengthwise of each other during the sliver-forming operation and cohering again after each re-arrangement. Fig. 3 shows a sliver formed in this manner from fibers as illustrated in Fig. 2. The sliver could be spun on spinning machines in the usual manner.

## Example II

20 kg. of palmetto fibers obtained by a mechanical defibration of the stems of scrub palmetto plants, as described in Example I, were boiled for 1 hour in a caustic soda solution of 5° Bé. strength. The color of the fibers darkened perceptibly but the fibers remained straight. At the end of the boiling period the fibers were washed with cold water and dried. On drying, kinks developed in the fibers substantially as shown in Fig. 2. The light brown kinky fibers were fed to a sliver-forming machine and formed into a spinnable sliver of the type illustrated in Fig. 3.

## Example III

A fiber mixture obtained by mechanical defibration of logs cut from the stems of scrub palmetto plants (*Serenoa repens*), as described in Example I, and containing longer fibers 10a and shorter fibers 10b (see Fig. 1), were separated by screening into short fibers 10b having a length up to 5 inches and long fibers 10a having a length between 5 inches and 14 inches (see flow diagram in Fig. 5). The long fibers 10a were treated with a tackifying agent and formed into

## 4

a light straw-colored spinnable sliver while tacky as described and claimed in my concurrently filed application.

50 kg. of the short fibers were placed in an iron vessel containing an aqueous caustic soda solution of 12° Bé. strength and boiled for 1 hour. At the end of this period the original light straw-color of the fibers had changed to a deep brown, but the fibers were still perfectly straight. The fibers were then removed from the lye, washed with lukewarm water which had been acidified by addition of hydrochloric acid to a pH value of 5.5 and left to dry. After drying, the fibers exhibited the hook-shaped kinks described in Example I and also a slight curl. The short kinky fibers were fed to a sliver-forming machine and formed into a brown, spinnable sliver of the type illustrated in Fig. 4. This sliver could spin into yarn on the usual spinning machines.

## Example IV

50 kg. palmetto fibers as obtained by a mechanical defibration of the stems of scrub palmetto plants (*Serenoa repens*), as described in Example I, were boiled for 2 hours in an aqueous caustic soda solution of 6° Bé. strength. After washing with cold water acidified with acetic acid to a pH value of 6.2, the fibers developed, on drying, the hook-shaped kinks illustrated in Fig. 2. They were then formed into a spinnable brownish colored sliver on a sliver-forming machine as described in Example I.

## Example V

35 20 kg. palmetto fibers as obtained from the mechanical defibration of the stems of scrub palmetto plants (*Serenoa repens*) as described in Example I were boiled for 2 hours in a caustic soda solution of 4° Bé. strength. After washing in warm water, and drying, the fibers which had developed a kinky appearance, substantially as shown in Fig. 2, were formed into a brownish spinnable sliver on a sliver-forming machine.

## Example VI

45 25 kg. of short palmetto fibers obtained from a mechanical defibration of the stems of scrub palmetto plants and subsequent separation of the long and short fibers, as described in Example III, were boiled for 10 minutes in a caustic soda solution of 30° Bé. strength. Then the fibers were washed in cold water and dried, developing during the drying kinks of the type described in the preceding examples. The light brown kinky fibers were fed to a sliver-forming machine and formed into a spinnable sliver, as shown in Fig. 4.

## Example VII

50 25 kg. of palmetto fibers obtained by a mechanical defibration of stems of scrub palmetto plants (*Serenoa repens*), as described in Example 1, were boiled for 10 minutes in a caustic soda solution of 55° Bé. strength. At the end of this period the fibers had assumed a medium brown color but were still straight. They were then washed with cold water acidified with acetic acid to a pH value of 6, and dried. During drying, the fibers became kinky, as shown in Fig. 2, and were then formed on a sliver-forming machine into a light brown spinnable sliver as shown in Fig. 3.

## Example VIII

55 20 kg. of palmetto fibers obtained by a mechanical defibration of stems of scrub palmetto plants (*Serenoa repens*), as described in Example

I, were boiled for 15 minutes in a caustic soda solution of 48° Bé. The dark brown fibers were then washed in cold water, acidified with hydrochloric acid to a pH value of 5.5, and dried. During drying, the fibers developed hook-shaped kinks, as shown in Fig. 2, and were then fed to a sliver-forming machine and formed into a dark brown spinnable sliver substantially as shown in Fig. 3.

I claim:

1. A process of preparing a brownish spinnable sliver from fibers contained in the stems of scrub palmetto plants (*Serenoa repens*), which process comprises the steps of boiling fibers obtained by a mechanical defibration of scrub palmetto plant stems for a period ranging from about 10 minutes to about 2 hours in an aqueous caustic soda solution of between about 4° and about 55° Bé. strength, the strength of the solution being related to the boiling time according to the formula:

$$a \times b = 5 \text{ to } 12$$

where  $a$  is the boiling time in hours and  $b$  is the strength of the solution in degrees Bé., washing the fibers with an aqueous medium having a pH value between about 5.5 and 7, drying them, the fibers developing during the drying hook-shaped kinks causing adjacent fibers to cohere together while being slidably displaceable lengthwise of one another, and forming the kinky fibers on a sliver-forming machine into a brownish spinnable sliver.

2. A process as claimed in claim 1, in which the fibers are boiled for about 30 minutes in a caustic soda solution of about 15° Bé. strength.

3. A process as claimed in claim 1, in which the fibers are boiled for about 1 hour in an aqueous caustic soda solution of about 5° Bé. strength.

4. A process of preparing a brownish spinnable sliver from fibers contained in the stems of scrub palmetto plants (*Serenoa repens*), which process comprises the steps of separating a mixture of

long and short fibers obtained by a mechanical defibration of scrub palmetto stems into short fibers having a length up to about 5 inches and long fibers having a greater length, boiling the short fibers for a period ranging from about 10 minutes to about 2 hours in an aqueous caustic soda solution of between about 4° and about 55° Bé. strength, the strength of the solution being related to the boiling time according to the formula:

$$a \times b = 5 \text{ to } 12$$

where  $a$  is the boiling time in hours and  $b$  is the strength of the solution in degrees Bé., washing the boiled fibers with an aqueous medium having a pH value between 5.5 and 7, drying them, the fibers developing during the drying hook-shaped kinks causing adjacent fibers to cohere together while being slidably displaceable lengthwise of one another, and forming the kinky fibers on a sliver-forming machine into a brownish spinnable sliver.

5. A process as claimed in claim 4, in which the fibers are boiled for about 1 hour in a caustic soda solution of about 12° Bé. strength.

BAREND GYSBERTUS HENRY  
VANDERJAGT.

#### REFERENCES CITED

The following references are of record in the file of this patent:

#### UNITED STATES PATENTS

| Number    | Name    | Date          |
|-----------|---------|---------------|
| 81,702    | Staufen | Sept. 1, 1868 |
| 203,177   | Miller  | Apr. 30, 1878 |
| 450,119   | Warrant | Apr. 7, 1891  |
| 1,051,124 | Kube    | Jan. 21, 1913 |

#### FOREIGN PATENTS

| Number  | Country       | Date          |
|---------|---------------|---------------|
| 356,754 | Great Britain | Sept. 7, 1931 |